

# United States Patent [19]

Warbichler, deceased et al.

[11] 3,816,190

[45] June 11, 1974

[54] **METHOD OF HEAT-TREATMENT OF ALUMINUM ALLOYS**

[76] Inventors: **Peter Warbichler, deceased**, late of Graz, Austria by Barbara Warbichler, heir; **Barbara Warbichler, Jr.**, Graz, Austria; **Ingrid Fraioli, nee Warbichler**, Graz, Austria; **Peter Warbichler, Jr.**, Graz, Austria heirs; **Firma Vereinigte Metallwerke Ranshofen-Berndorf Aktiengesellschaft**, Ranshofen, Austria

[22] Filed: **May 22, 1972**

[21] Appl. No.: **255,511**

**Related U.S. Application Data**

[63] Continuation-in-part of Ser. No. 806,926, March 13, 1969, abandoned.

[52] **U.S. Cl.** ..... **148/159**, 148/11.5 R, 148/12.7

[51] **Int. Cl.** ..... **C22f 1/04**

[58] **Field of Search** ..... 148/11.5, 12.7, 159

[56] **References Cited**

UNITED STATES PATENTS

2,695,253 11/1954 Schaaber ..... 148/159

|           |         |                  |          |
|-----------|---------|------------------|----------|
| 3,135,633 | 6/1964  | Hornus .....     | 148/159  |
| 3,222,227 | 12/1965 | Bough et al..... | 148/11.5 |
| 3,379,583 | 4/1968  | Gruhl et al..... | 148/11.5 |
| 3,418,177 | 12/1968 | Pryor .....      | 148/11.5 |

*Primary Examiner*—Charles N. Lovell

[57]

**ABSTRACT**

A method of heat treatment of aluminum alloys of the type Al-Mg-Si for the purpose of improvement of the processibility by extruding, which comprises the steps of subjecting said alloys to a homogenization-glowing at 530°C to 580°C, and cooling and alloys to a temperature range of 230°C to 270°C, while maintaining a substantially uniform temperature gradient. The cooling step takes place at a speed of at least 100°C/h without quenching, and a holding period is maintained within the temperature range of 230°C to 270°C, for a time period of about 4 to 24 hours, whereupon further cooling or heating to working temperature of said alloys is performed.

**6 Claims, 2 Drawing Figures**

PATENTED JUN 11 1974

3,816,190

SHEET 1 OF 2



FIG. 1

PATENTED JUN 11 1974

3,816,190

SHEET 2 OF 2



FIG. 2

## METHOD OF HEAT-TREATMENT OF ALUMINUM ALLOYS

The present invention is a continuation-in-part of the co-pending patent application Ser. No. 806,926, filed Mar. 13, 1969 now abandoned.

The present invention relates to a method of heat treatment of aluminum alloys having the DIN characteristics AlMgSi 0.5 dek and AlMgSi 1, respectively, which have the following compositions: Mg 0.4 - 0.9 and 0.6 - 1.4, respectively; Si 0.3 - 0.7 and 0.6 - 1.6, respectively; Fe 0.4 and 0.5, respectively; Mn 0.3 and 1.0, respectively; Cr 0.05 and 0.3, respectively. The rest is remainder of aluminum and unavoidable impurities.

The heat treatment in accordance with the present invention has the purpose to improve the processibility characteristics of the mentioned alloys in extruders.

Methods for heat treatment of alloys of the type of AlMgSi are known in which the material is subjected to a conventional homogenizing glowing within the range of 530°C - 580°C, whereupon the material cools off with a temperature gradient of less than 50°C/h, preferably of 20°C/h to about 250°C. The thus treated materials can then be heated up to a hot fabrication temperature of 350°C to 530°C for the purpose of extruding. In this treatment, many of the dissolved ingredients of Mg and Si can be precipitated in coarse form.

It is not the aim of the present invention to obtain such structure. During the investigations, which have guided to the present invention, it has been found rather, that the desired improvement of the processibility characteristics are obtained then particularly for extruding when possibly many of the solved ingredients of Mg and Si are separated in form of finest particles, which are to a great extent coherent with the Al matrix and during heating to extensive temperature do not go completely in solution, but rather break during the molding and during the following hot settling can be effective as a nucleus for the precipitation.

It is one object of the present invention to provide a method for heat treatment of aluminum alloys, wherein the alloys in conventional manner are subjected to a homogenizing glowing at 530°C - 580°C, and thereafter are cooled by maintaining a substantially uniform temperature gradient to a temperature within the range of 230°C to 270°C, the cooling taking place at a speed of at least 100°C/h, (or cooled by maintaining a substantially uniform temperature gradient to a temperature within the range of room temperature to 270°C) however, with the avoidance of a quenching, whereupon a holding time is injected in the mentioned temperature range of 230°C to 270°C, or of room temperature to 270°C for a time period of 4 to 24 hours, and the alloys are then cooled, if desired, or permitted to cool, or are heated to working temperature.

It has been found that a complete structural change in the desired direction is obtained after a holding of about 8 h. In case of longer holding in the mentioned range, in other words no essential or appreciable structure change takes place any more. For some working purpose, however, already, a part structural variation of the desired type is sufficient: in such cases, shorter holding time periods can suffice.

If desired, the glowing and the following tempering can be repeated under circumstances during different time periods.

In this connection it should be mentioned that one cools from the given glowing temperature to the room temperature and thereafter to heat up again to tempering temperature; however, this variation of the heat treatment requires totally rather long treatment times.

With these and other objects in view, which will become apparent in the following detailed description, the present invention will be clearly understood in connection with the accompanying drawing, in which:

FIG. 1 is a 2100 times enlargement of a testing material; and

FIG. 2 is an enlargement of the surface structure obtained by applying the method of the present invention.

Referring now to FIG. 1, a 2100 times enlargement of a tube consisting of an Al-Mg-Si-alloy of the type marked as P 568 is disclosed. The surface has been as conventional metallographically preworked, electro-polished and chemically etched. The photo has been made in an emission electron microscope. The heat treatment of the sample has been performed in accordance with the statements given in the German patent publication No. 1,247,030, namely one hour at 570°C to 580°C homogenized, thereafter cooled within 330 minutes down to 300°C (temperature gradient 50°C/h) and thereafter cooled off in air. The structure of the surface shows comparatively few irregularly distributed material separations.

Referring now to FIG. 2, the preparation of the sample shown therein took place in the same manner as disclosed in connection with FIG. 1, with the same material. The heat treatment consisted of a homogenization for one hour at 570°C to 580°C. Thereafter, the sample has been cooled off within 60 minutes to about 250°C (temperature gradient of at least 100°C/h). Thereafter, for 24 hours the temperature was maintained at 250°C and then cooling off took place in the air. Referring again to FIG. 2 of the drawings, the surface structure is completely different from that obtained in the known methods. One recognizes the fine uniform needle-like characterized separations divided over the entire surface, which separations correspond with the above-stated requirements. It is, undoubtedly apparent, that the compared methods differ from each other not only formally, but lead metallurgically to completely different results.

It is to be understood, that in case longer treatment time periods are taken in stride, the indicated temperature ranges of the glowing and of the tempering can be undercut. Such measures do not bring about basically and economically advantages, are, however, within the frame work of the present invention.

While we have disclosed one embodiment of the present invention it is to be understood that this embodiment is given by example only and not in a limiting sense.

We claim:

1. A method of heat treatment of aluminum alloys of the type Al-Mg-Si for the purpose of improvement of the processibility by extruding, comprising the steps of

subjecting said alloys to a homogenization-glowing at 530°C to 580°C,  
cooling said alloys to a temperature within the range of 230°C to 270°C, while maintaining a substantially uniform temperature gradient,

said cooling step taking place at a speed of at least 100°C/h without quenching, maintaining a holding period of about 4 to 24 hours within said temperature range of 230°C to 270°C, and further cooling said alloys.

2. The method, as set forth in claim 1, wherein said holding period is maintained for about 8 hours.

3. The method, as set forth in claim 1, wherein said holding period is maintained for about 24 hours.

4. A method of heat treatment of aluminum alloys of the type Al-Mg-Si for the purpose of improvement of the processibility by extruding, comprising the steps of subjecting said alloys to a homogenization-glowing at

530°C to 580°C, cooling said alloys to a temperature within the range of 230°C to 270°C, while maintaining a substantially uniform temperature gradient,

5 said cooling step taking place at a speed of at least 100°C/h without quenching, maintaining a holding period of about 4 to 24 hours within said temperature range of 230°C to 270°C, and

10 heating to extrusion working temperature of said alloys.

5. The method, as set forth in claim 4, wherein said holding period is maintained for about 8 hours.

6. The method, as set forth in claim 4, wherein said holding period is maintained for about 24 hours.

\* \* \* \* \*

20

25

30

35

40

45

50

55

60

65

UNITED STATES PATENT OFFICE  
CERTIFICATE OF CORRECTION

Patent No. 3,816,190

Dated June 11, 1974

Inventor(s) Peter Warbichler, deceased, by Barbara Warbichler  
et al.

It is certified that error appears in the above-identified patent  
and that said Letters Patent are hereby corrected as shown below:

On the cover sheet item [76] cancel the assignee's  
name from the names of the inventors, and insert,  
--[73] Assignee: Firma Vereinigte Metallwerke Ranshofen-  
Berndorf Aktiengesellschaft, Ranshofen,  
Austria --.

Signed and sealed this 1st day of October 1974.

(SEAL)

Attest:

McCOY M. GIBSON JR.  
Attesting Officer

C. MARSHALL DANN  
Commissioner of Patents

UNITED STATES PATENT OFFICE  
CERTIFICATE OF CORRECTION

Patent No. 3,816,190 Dated June 11, 1974

Inventor(s) Peter Warbichler, Deceased

It is certified that error appears in the above-identified patent and that said Letters Patent are hereby corrected as shown below:

On the Title page, in item 76 "Ingrid Fraioli, nee Warbichler" should read -- Ingrid Fraioli, nee Warbichler

and the assignee should read: -- Firma Zentrum Fur Elektronenmikroskopie, Austria (and) Firma Vereinigte Metallwerke Ranshofenberndorf Aktiengesellschaft, Austria -

Item 54 should read:--Method Of Heat-Treatment Of Aluminum Alloys--

Signed and sealed this 7th day of January 1975.

(SEAL)

Attest:

McCOY M. GIBSON JR.  
Attesting Officer

C. MARSHALL DANN  
Commissioner of Patents